

# UNITED STATES PATENT OFFICE.

RENÉ CLAVEL, OF BASEL-AUGST, SWITZERLAND.

## PROCESS FOR DYEING CELLULOSE ACETATES.

1,378,443.

Specification of Letters Patent.

Patented May 17, 1921.

No Drawing.

Application filed January 5, 1921. Serial No. 435,225.

To all whom it may concern:

Be it known that I, RENÉ CLAVEL, a citizen of the Swiss Republic, and resident of Basel-Augst, Switzerland, have invented a new and useful Process for Dyeing Cellulose Acetates, of which the following is a full, clear, and exact specification.

It is known that cellulose acetate, such as cellulose acetate silks, cellulose acetate films and the like cannot be directly dyed in practice by the usual dyeing methods such as are used, for example, for artificial silk, because the power of taking up the dyestuff is completely or essentially lacking.

There are various processes for treating cellulose acetate silks and cellulose acetate films with inorganic or organic compounds before they are dyed, in order to increase the capacity of the fiber for taking up the dye in the dyeing operation. None of these processes has found technical application in the art because such preliminary treatment gives rise to tendering and loss of the cellulose acetate. Furthermore, treatment with alkalis at high temperatures gives rise to undesirable losses in the luster of the cellulose acetates under treatment.

The present invention relates to a process for directly dyeing cellulose acetates, cellulose acetate silks and cellulose acetate films, consisting in dyeing them with acid, basic or direct dyestuffs, preferably with addition of one or more protective colloids such as gelatin or gelatin soaps, in presence of a weak acid, preferably an organic acid like acetic acid or formic acid, and in presence of at least one chlorid soluble in water, such as a chlorid like stannous chlorid, zinc chlorid, magnesium chlorid, or ammonium chlorid. In this manner, the cellulose acetates in the form of bands or of threads may be dyed at temperatures up to boiling temperature without depreciation of luster and without the usual losses, woolly effects, tendering and the like, due, for instance, to saponification.

For example, the acid dye solutions containing one or more dyes may contain chlorid of zinc, of potassium, of sodium, of magnesium, or of barium, or a mixture of them, in presence of one or more protective colloids such as gelatin, albumen, boiled-off liquors, a tannate, or saponified or sulfonated fatty acids. The dyestuffs which may be used are any basic, acid or direct dyeing dyestuffs. The dyeing is performed in a liquid bath, preferably in foam, as described in the specification of U. S. Letters Patent

No. 1234732 dated July 31, 1917, in which case the protective colloids together with the salt solution serve at the same time as emulsifiers and foam producers and by their surface activity in common with the color-colloids considerably increase the power of absorption of the cellulose acetate.

### Example.

65

1 kilo of cellulose acetate silk is suspended in a foam apparatus. To the color bath of about 20-30 liters, which is beneath the suspended silk, are added 300 cubic centimeters of formic acid, 100-1000 gms. of zinc chlorid and 12 gms. of glue and the whole is heated to 50° C. The liquid is then converted into foam which surrounds the cellulose acetate silk on all sides; after a quarter of an hour the bath is heated to boiling and the goods are left in position for another quarter of an hour. The dyeing is continued until up to the sample, if necessary with a further addition of dyestuff, and the goods are washed for a short time in a bath of soft water containing an oil emulsion.

70

75

What I claim is:

1. The herein described process for dyeing cellulose acetates, consisting in carrying out the dyeing operation with a dyestuff-solution, which contains a weak acid and at least one soluble chlorid.

2. The herein described process for dyeing cellulose acetates, consisting in carrying out the dyeing operation with a dyestuff-solution which contains a weak acid, at least one soluble chlorid and at least one protective colloid.

3. The herein described process for dyeing cellulose acetates, consisting in carrying out the dyeing operation with a dyestuff-solution, which contains an organic acid and at least one soluble chlorid.

4. The herein described process for dyeing cellulose acetates, consisting in carrying out the dyeing operation with a dyestuff-solution which contains an organic acid, at least one soluble chlorid and at least one protective colloid.

100

In witness whereof I have hereunto signed my name this eleventh day of December, 1920, in the presence of two subscribing witnesses.

105

RENÉ CLAVEL.

Witnesses:

FRIDA SALAODIN,  
ARMAND RITTER,